

Dec. 25, 1951

E. G. L. ROBERTS

2,580,244

MINERAL INSULATED CONDUCTOR WORKPIECE

Filed Oct. 15, 1947



Inventor  
Edwin G. L. Roberts  
By  
A. Knight Board  
Attorney

## UNITED STATES PATENT OFFICE

2,580,244

MINERAL INSULATED CONDUCTOR  
WORKPIECEEdwin Gilbert Llewellyn Roberts,  
Bolton, EnglandApplication October 15, 1947, Serial No. 779,912  
In Great Britain October 24, 1946

4 Claims. (Cl. 174—77)

1

This invention relates to the manufacture of metal clad electric conductors and more particularly to an article of manufacture adapted to be used as initial work-piece in a process for the manufacture of metal clad mineral insulated conductors by the reduction in cross-section of such initial work-piece.

The object of the present invention is to provide an article of manufacture which will overcome the objections referred to. According to the present invention the article of manufacture comprises in combination a metal tube, a granular dielectric crypto-crystalline material consisting of gamma alumina filling the metal tube, the granular dielectric crypto-crystalline material being isotropic and amorphous and possessing plastic and fluid properties, and means closing at both ends the metal tube filled with the granular dielectric crypto-crystalline material.

In the accompanying drawing which illustrates one embodiment of this invention:

Figure 1 is a vertical section of a tubular body fitted with a pair of conductor rods.

Figure 2 is a similar view illustrating the body partially filled with insulating material or dielectric, and the ram used for pressing the same into a compact condition.

Figure 3 is a similar view illustrating the body filled to the desired extent and with a metallic sealing disc in position, and

Figure 4 is a similar view illustrating the means for closing the end of the tubular body over the top of the sealing disc and for bringing the insulating material up to the required density for its occupied volume.

In the drawings, which illustrate an embodiment of the invention as applied to a work-piece provided with two conducting rods designed in the completed conductor to be insulated from each other, the work-piece comprises a metallic tube or bottle 1, the closed end 2 of which is drilled and tapped to receive the threaded ends of the conductor rods 3 suitably spaced apart. The open end of the tube 1 is bevelled as at 4 on the inside for the purpose hereafter described.

In carrying out this invention the work-piece comprising the tube 1 and conductor rods 3 is loaded with insulating material or dielectric 5 consisting of gamma alumina, which material as before stated is isotropic or amorphous, and is in a granular form, such material being hereinafter referred to as the dielectric material. After a given quantity of material has been fed into the tube it is partially consolidated in situ by a suitable ram 6 provided on its lower end with a die 7.

2

Then the ram is withdrawn and further quantities of the dielectric are fed in and partially consolidated until the tube is practically filled, allowing sufficient length at the open end, as illustrated in Figure 3, to permit a metallic disc 8 suitably drilled to be placed over the conductors 3, and, by affixing a suitably formed die 9 on to the end of the ram 6 to close over on to said disc the bevelled end 4 of the tube and thereby lock the sealing disc 8 firmly in position on top of the dielectric material 5, said dielectric material being simultaneously consolidated to maximum density for its occupied volume by pressure. The dielectric material is normally obtained in commerce in the form of a finely divided powder, and requires treatment before it is suitable for the purposes of my invention. A convenient method of bringing the finely divided powder into the granular form is first to agglomerate the same by dry pressing or moulding as is common in ceramic technique and then to disintegrate the same by a crushing operation designed to reduce it to an aggregate so that the particles will pass through a circular aperture of approximately one-quarter of an inch in diameter. The completed work-piece can be drilled with small holes at both ends to enable the free egress of water (if any) vapour and gases, when it is heated. In cases where hot rolling of the work-piece is required, said work-piece can be either dried to expel the mechanically held or chemically combined water and occluded gases previous to heating to the necessary temperatures required to roll it in the hot condition, or, it can be slowly heated up to that temperature in one operation. Such rolling temperature ranges from 800° to 900° C. in the case of copper sheaths and conductors.

What I claim is:

1. An article of manufacture adapted to be used as initial work-piece in a process for the manufacture of metal clad mineral insulated conductors by the reduction in cross-section of such initial work-piece, said article of manufacture comprising in combination, a metal tube; a granular dielectric crypto-crystalline material consisting of gamma alumina filling said metal tube, said granular dielectric crypto-crystalline material being isotropic and amorphous and possessing plastic and fluid properties; and means closing at both ends said metal tube filled with said granular dielectric crypto-crystalline material.
2. An article of manufacture adapted to be used as initial work-piece in a process for the manufacture of metal clad mineral insulated

conductors by the reduction in cross-section of such initial work-piece, said article of manufacture comprising in combination, a metal tube; granular gamma alumina filling said metal tube; and closing means closing at both ends the metal tube filled with said granular gamma alumina.

3. An article of manufacture adapted to be used as initial work-piece in a process for the manufacture of metal clad mineral insulated conductors by the reduction in cross-section of such initial work-piece, said article of manufacture comprising in combination, a metal tube being open at one end and composed of a metal cylindrical wall and a metal end wall provided at one end of said metal cylindrical wall and forming one unitary structure with said metal cylindrical wall of said metal tube closing the same at its other end; a granular dielectric crypto-crystalline material consisting of gamma alumina filling said metal tube, said granular dielectric crypto-crystalline material being isotropic and amorphous and possessing plastic and fluid properties; and closure means closing said open end of said metal tube filled with said granular dielectric crypto-crystalline material.

4. An article of manufacture adapted to be used as initial work-piece in a process for the manufacture of metal clad mineral insulated conductors by the reduction in cross-section of such initial work-piece, said article of manufacture comprising in combination, a metal tube being open at one end and composed of a metal cylindrical wall and a metal end wall provided at one end of said metal cylindrical wall and forming one unitary structure with said metal cylindrical wall of said metal tube closing the same at its other end; a granular dielectric crypto-crystalline material consisting of gamma

alumina filling said metal tube, said granular dielectric crypto-crystalline material being isotropic and amorphous and possessing plastic and fluid properties; closure means closing said open end of said metal tube filled with said granular dielectric crypto-crystalline material; at least one opening in said closure means; and at least one core arranged within said metal tube extending in longitudinal direction thereof secured at one end to said metal end wall of said metal tube and passing at its other end through said opening in said closure means closing said open end of said metal tube.

EDWIN GILBERT LLEWELLYN ROBERTS.

#### REFERENCES CITED

The following references are of record in the file of this patent:

#### UNITED STATES PATENTS

| Number    | Name      | Date           |
|-----------|-----------|----------------|
| 573,176   | Borel     | Dec. 15, 1896  |
| 1,127,281 | Read      | Feb. 2, 1915   |
| 1,157,916 | Wentworth | Oct. 26, 1915  |
| 1,192,457 | Read      | July 25, 1916  |
| 1,279,252 | Capp      | Sept. 17, 1918 |
| 1,809,089 | Wiegand   | June 9, 1931   |
| 1,993,580 | Abbott    | Mar. 5, 1935   |
| 2,091,839 | Tangeman  | Aug. 31, 1937  |
| 2,123,778 | Heilmann  | July 12, 1938  |
| 2,279,726 | Allen     | Apr. 14, 1942  |
| 2,431,474 | Gandenzi  | Nov. 25, 1947  |

#### OTHER REFERENCES

35 Tomlinson et al.: Publication entitled "Mineral-Insulated Metal-Sheathed Conductors;" Journal of the Institute of Elect. Engrs.; August 1946; pgs. 325-340; pg.325 in particular relied upon. Copy in Div. 65.